# EUROPEAN PATENT SPECIFICATION

(11) **EP 0 917 594 B1**
(45) Date of publication and mention of the grant of the patent: **29.11.2000**
(21) Application number: 97941934.8
(22) Date of filing: 08.08.1997
(51) Int. Cl.: C22C 38/06, C22C 38/00

(54) **STEEL, METHOD FOR ITS MANUFACTURE, ITS USE AND PRODUCT MADE FROM STEEL**
STAHL, HERSTELLUNGSVERFAHREN, VERWENDUNG UND GEGENSTAND, AUS DIESEN STAHL HERGESTELLT
ACIER, PROCEDE DE FABRICATION DE CET ACIER, UTILISATION DE CET ACIER ET PRODUITS FAITS DE CET ACIER

(30) Priority: 08.08.1996 NL 1003762
(43) Date of publication of application: 26.05.1999
(73) Proprietor: Corus Staal BV, 1970 CA Ijmuiden (NL)
(72) Inventor: JONKER, Frederik, NL-1963 CA Heemskerk (NL); SCHOL, Willem, Jan, NL-1827 PJ Alkmaar (NL); MULDER, Johannes, NL-1943 BG Beverwijk (NL); DE HAAS, Maarten, Arie, NL-1702 KK Heerhugowaard (NL); JANSEN, Egbert, NL-1446 CT Purmerend (NL)
(74) Representative: Herman de Groot, Johan Willem
(86) International application number: EP9704407
(87) International publication number: WO9806881

(56) References cited:
- EP-A- 0 592 267
- EP-A- 0 612 857
- FR-A- 2 179 008
- GB-A- 1 384 331
- US-A- 4 348 229

## Description

### Field of the invention

The invention relates to a steel in the form of sheet or strip with excellent stretching and deep-drawing and wall ironing properties, in particular for packaging applications, a method for its manufacture and also a use of such a steel. In the context of this application the packaging steel is taken to mean a consecutively hot-rolled, pickled, cold-reduced, annealed and generally temper-rolled or further cold-reduced steel in the form of sheet or strip whether or not coiled. Blanks of this sheet or strip are to be made in a number of forming operations into a (semi-finished) product for example a beverage can or other object, whereby for the purposes of the intended shape, the flat basic material needs to undergo extensive material deformations. For manufacturing a beverage can a cup is formed for example by deep drawing from a blank of packaging steel in one or more stages, the walls of which are wall-ironed in order to give the can thus formed a greater height/content. In particular the deep-drawing in one stage and wall-ironing require an easily formable material that has ideally isotropic properties.

### Summary of the invention

In this connection and also within the broader scope of continuous endeavours to improve the said steel grades, the search is directed in particular towards a combination of the following properties:
- high r-value (Lankford-value);
- as small as possible differences in mechanical properties across above all the strip width, but also along the strip length, in specialist terms low spread of the properties "edge/centre" and "along the coil" respectively.

Experiments now show that a steel grade displaying spectacularly better uniform mechanical properties - in annealed and optionally further cold reduced, e.g. temper-rolled condition - is found if the steel has the composition:

| Element | Min* | Max* |
|---|---|---|
| C | | 40 |
| Mn | 140 | 250 |
| P | | 20 |
| S | | 20 |
| Si | | 30 |
| N ppm | | 30 |
| Al ** | | 50 |
| B ppm | 5 | 50 |
| Cu | | 40 |
| Sn | | 10 |
| Cr | | 40 |
| Ni | | 40 |
| Mo | | 10 |

| | | |
|---|---|---|
| * in 0.001 % wt. unless otherwise stated | | |
| ** acid soluble | | |

balance Fe and inevitable impurities, wherein 0.4 ≤ B / N ≤ 1.2, wherein the grain size in an edge region of the strip Gs-edge and the grain size in a centre region of the strip Gs-centre differ less than 0.5 ASTM units.

This steel makes it possible to attain an improved level of stretching, deep-drawing and wall ironing properties and a greatly reduced spread of the mechanical properties.

It is preferred that the composition complies with:

| Element | Min* | Max* |
|---|---|---|
| C | 10 | 40 |
| Mn | 140 | 200 |
| P | | 20 |
| S | | 20, preferably 10 |
| Si | | 30 |
| N ppm | | 25 |
| Al ** | 15 | 35 |
| B ppm | 8 | 25 |
| Cu | | 40 |
| Sn | | 10 |
| Cr | | 40 |
| Ni | | 40 |
| Mo | | 10 |

| | | |
|---|---|---|
| * in 0.001 % wt. unless otherwise stated | | |
| ** acid soluble | | |

It is found that to achieve optimum results in accordance with the invention within the limits indicated above the following target values can be given:

| Element | Target* +/- 30 % |
|---|---|
| C | 20 |
| Mn | 160 |
| N ppm | 20 |
| Al ** | 25 |
| B ppm | 0.8.N |

| | |
|---|---|
| * in 0.001 % wt. unless otherwise stated | |
| ** acid soluble | |

Because better mechanical properties can be obtained in accordance with the invention it is possible to select a thinner material of thinner than 0.35 down to even thinner than 0.18 mm, which fits in excellently with the search to apply lighter weight for example for a steel beverage can.

It is particularly advantageous if the steel strip is in the form of cold reduced, annealed and optionally further cold reduced strip or sheet wherein the grain size in an edge region of the strip Gs-edge and the grain size in a centre region of the strip Gs-centre differ less than 0.5 ASTM units, respectively wherein the r-value in an edge region of the strip r-edge and the r-value in a centre region of the strip r-centre differ less than 0.2 units, preferably less than 0.1 units, respectively wherein the Yield Point in an edge region of the strip Rp-edge and the Yield Point in a centre region of the strip Rp-centre differ less than 20 N/mm², respectively wherein the average r-value is at least 1.3.

The production of stretched, deep drawn and drawn and wall ironed products from blanks cut from the steel according to the invention can be carried out much more efficiently with lower spoilage.

The invention is further embodied in a method for manufacturing an annealed steel strip from the steel according to any one of claims 1-7, comprising the stages:
- hot-rolling comprising finish-rolling at a finish-rolling temperature and coiling at a coiling temperature;
- pickling;
- cold-rolling;
- annealing, preferable, continuous annealing;
- and optionally further cold rolling, preferably with a reduction of at least 0.6 %;
wherein the finish-rolling temperature is selected above Ar₃-10 °C and the coiling temperature is selected below 700 °C.

In a preferred method the finish-rolling temperature is selected above 825 °C and the coiling temperature below 690 °C, more preferably the finish-rolling temperature is selected at 900 ± 30 °C and the coiling temperature at 670 °C ± 20 °C.

In the method preferably the total cold reduction before annealing is 85 % or more.

In an aspect of the method according to the invention further cold rolling after annealing is carried out with a reduction of > 5 %, or even with a reduction of 10-20 %.

This creates a steel strip with very good forming properties. In the case of further cold rolling after annealing, e.g. temper rolling it is preferable to do so with a reduction of at least 0.6 %. Preferably a target value is selected for the finish-rolling temperature of 900°C and for the coiling temperature a target value of 670°C. This establishes the basis for a very easily workable, homogeneous steel sheet. It is preferable that if temper-rolling is carried out it is done so in accordance with the invention with a reduction of 10-20 %. Such a high degree of deformation still produces a steel grade with excellent mechanical properties.

The steel grade in accordance with the invention is found to be perfectly suitable for application as packaging steel in drawing and wall-ironing (DWI) applications, for example applications wherein the packaging steel is coated with a coating comprising Sn and afterwards subjected in succession to deep-drawing and wall-ironing as in the manufacture of the body part of a two-piece can.

The excellent mechanical properties of the steel allow such a can to be made even lighter, again responding to the demand for increasingly less material consumption and weight for packaging and other products.

The invention is also embodied in a use of the steel for stretching, deep-drawing and drawing and wall-ironing applications, in a steel provided with one or more coatings selected from the group of coatings comprising Sn, Cr, lacquer, organic coating, polymer and combinations thereof on one or both sides of the strip or sheet, and in a stretched, deep drawn or drawn and wall ironed product made from steel according to the invention.

The invention will now be illustrated by reference to the results of some experiments further details of which are given in the following tables 1 to 5.

In the experiments continuously cast steel was hot rolled in a hot rolling mill with a finish-rolling temperature of 900 °C and coiled at coiling temperatures with target values of 625, 670 and 690 °C. Subsequently the steel was pickled in a conventional pickling line and cold rolled with a reduction of 88-89 %. Thereafter it was continuously annealed. After annealing further cold reduction was performed either temper rolling with a reduction of 0.8 % or cold rolling with a reduction of 4 % and 6 %. The steel was then tinned in a conventional electrolytic tinning line.

**Table 1**

| Steel tested Chemical composition in 0.001 wt. % and wt. ppm where stated | | | | | | | | |
|---|---|---|---|---|---|---|---|---|
| Steel | C | Mn | S | Al* | B ppm | N ppm | CT (°C) | Remarks |
| A | 24 | 202 | 7 | 26 | 16 | 24 | 625 | invention |
| B | 23 | 191 | 7 | 34 | 20 | 29 | 690 | invention |
| C | 16 | 171 | 5 | 28 | 8 | 22 | 690 | invention |
| D | 25 | 200 | <12 | 35 | - | 20 | 670 | comparative |

| | | | | | | | | |
|---|---|---|---|---|---|---|---|---|
| Al * : Aluminium acid soluble CT : Coiling temperature after hot rolling | | | | | | | | |

**Table 2**

| Chemical composition of steel C, in hot rolled condition in 0.001 wt. % and wt. ppm where stated | | | | | | | |
|---|---|---|---|---|---|---|---|
| Position | C | Mn | Al* | B ppm | B *ppm | N ppm | N * ppm |
| Strip centre | 16 | 171 | 28 | 8 | 1 | 22 | < 2 |
| Strip edge | 16 | 173 | 28 | 8 | 1 | 17 | < 2 |

| | | | | | | | |
|---|---|---|---|---|---|---|---|
| Al * : Aluminium acid soluble | | | | | | | |
| B * : Boron acid soluble | | | | | | | |
| N * : Nitrogen not bound | | | | | | | |

**Table 3**

| Grain size of steel C, in hot rolled and in cold-rolled, annealed condition | | |
|---|---|---|
| Position | Grain size (ASTM) | |
| | Hot rolled | Cold rolled |
| Strip centre | 9.0 | 11.5 |
| Strip edge | 9.0 | 11.5 |

**Table 4**

| Mechanical properties of steel C in cold-rolled, annealed, temper rolled (reduction 0.8 %) condition | | | | | |
|---|---|---|---|---|---|
| Position | | Strip centre | | | strip edge |
| Direction | | lengthwise | oblique | widthwise | lengthwise |
| r-value | test 1 | 1.57 | 1.68 | 1.83 | 1.49 |
| | test 2 | 1.58 | 1.68 | 1.80 | 1.49 |
| | test 3 | 1.58 | 1.80 | 1.82 | 1.42 |
| | average | 1.58 | 1.72 | 1.82 | 1.47 |
| Reh (Rp) | test 1 | 237 | 234 | 236 | 247 |
| | test 2 | 238 | 235 | 235 | 247 |
| | test 3 | 238 | 235 | 235 | 247 |
| | average | 238 | 235 | 235 | 247 |
| Rm | test 1 | 360 | 354 | 359 | 358 |
| | test 2 | 362 | 354 | 356 | 358 |
| | test 3 | 362 | 356 | 358 | 357 |
| | average | 361 | 355 | 358 | 358 |

In the above table 4 the r-value means the Lankford-value, Reh (Rp) the yield point in N/mm², Rm the tensile strength in N/mm².

The small differences between the values in one row show that the mechanical properties across the width of the sheet vary little.
Notable is the high r-value but particularly the small difference in properties per indicated direction, where 'lengthwise' means in the direction of rolling, 'oblique' at 45° to it and 'widthwise' perpendicular to it, more particularly the small difference in properties between the properties of centre portions and edge portions.

**Table 5**

| Yield Point and Grain size of steels A, B and D in annealed, temper rolled (reduction 0.8 %) condition | | | | | |
|---|---|---|---|---|---|
| Steel | Yield Point in N/mm² | | ASTM | | Remark |
| | centre | edge | centre | edge | |
| A | 258 | 256 | 11 | 11 | invention |
| B | 237 | 235 | 11 | 11 | invention |
| D | 262 | 265 | 11 | 12 | comparative |

**Table 6**

| Table 6 Yield Point of steels B and D in annealed, rolled condition with different reductions after annealing | | | |
|---|---|---|---|
| Steel | cold reduction after annealing in % | Yield Point in N/mm² | |
| | | centre | edge |
| B | 1 | 231 | 233 |
| B | 4 | 283 | 281 |
| B | 6 | 330 | 333 |
| D | 1 | 258 | 268 |

In a comparative test steels C and D of table 1 were tested on behaviour and performance in a heavy forming operation. Hereto tin plated circular blanks all of the same diameter from head, tail and in between portions taken from centre, edge and in between regions of the strip were drawn into cups which cups were wall ironed, trimmed and pre-spin-necked. The pre-spin-necked cans thus obtained were of the type that are to be made into the commonly used and well known 33 cl. beverage can having a diameter of 66 mm. Of the pre-spin-necked cans the dimensions pre-spin edge diameter PSED (mm) and pre-spin plug diameter PSPD (mm) were determined. Reference is made to the drawings.

### Description of the drawings

Fig. 1 shows the relevant dimensions PSED and PSPD discussed above, and
Fig. 2 is a graph showing the relation PSED vs. PSPD.

In Fig. 1 a pre-spin-necked can is shown. The can is formed with a neck which is of smaller diameter than its main body portion, this neck having a cylindrical portion of diameter PSPD and an out-turned flange at its end having a maximum diameter PSED as indicated in Fig. 1. These diameters are dependent on the material quality but are critical for successful can formation, since the neck is used to fix the lid in place after filling.

In Fig. 2 each open square symbol indicates the values of PSED and PSPD of a pre-spin-necked can made from a blank taken from the steel C according to the invention and each filled square symbol indicates those of a can made from comparative steel D. The vertical line at a PSED value of in this case 56.1 indicates the limit for PSED above which the manufactured can will be rejected because of wavy flanges.

The results clearly show the two effects of using steel according to the invention. Firstly the spread in PSED and PSPD and thus in material properties is smaller for cans made from steel according to the invention and secondly it turns out that the cans made from steel according to the invention show a lower PSED value and consequently a lower reject rate.

## Claims

1. Steel in the form of cold reduced, annealed and optionally further cold reduced sheet or strip having a chemical composition:
| Element | Min* | Max* |
|---|---|---|
| C | | 40 |
| Mn | 140 | 250 |
| P | | 20 |
| S | | 20 |
| Si | | 30 |
| N ppm | | 30 |
| Al ** | | 50 |
| B ppm | 5 | 50 |
| Cu | | 40 |
| Sn | | 10 |
| Cr | | 40 |
| Ni | | 40 |
| Mo | | 10 |
| | | |
|---|---|---|
| * in 0.001 % wt. unless otherwise stated | | |
| ** acid soluble | | |
balance Fe and inevitable impurities, wherein 0.4 ≤ B / N ≤ 1.2, wherein the grain size in an edge region of the strip Gs-edge and the grain size in a centre region of the strip Gs-centre differ less than 0.5 ASTM units.

2. Steel according to claim 1 having a chemical composition:
| Element | Min* | Max* |
|---|---|---|
| C | 10 | 40 |
| Mn | 140 | 200 |
| P | | 20 |
| S | | 20, preferably 10 |
| Si | | 30 |
| N ppm | | 25 |
| Al ** | 15 | 35 |
| B ppm | 8 | 25 |
| Cu | | 40 |
| Sn | | 10 |
| Cr | | 40 |
| Ni | | 40 |
| Mo | | 10 |
| | | |
|---|---|---|
| * in 0.001 % wt. unless otherwise stated | | |
| ** acid soluble | | |

3. Steel in accordance with Claim 1 or Claim 2, wherein for the following elements the following standard values are respected:
| Element | Standard* +/- 30 % |
|---|---|
| C | 20 |
| Mn | 160 |
| N ppm | 20 |
| Al ** | 25 |
| B ppm | 0.8.N |
| | |
|---|---|
| * in 0.001 % wt. unless otherwise stated | |
| ** acid soluble | |

4. Steel in accordance with any one of the preceding claims in the form of cold reduced, annealed and optionally further cold reduced strip or sheet wherein the r-value in an edge region of the strip r-edge and the r-value in a centre region of the strip r-centre differ less than 0.2 units, preferably less than 0.1 units.

5. Steel in accordance with any one of the preceding claims in the form of cold reduced, annealed and optionally further cold reduced strip or sheet wherein the Yield Point in an edge region of the strip Rp-edge and the Yield Point in a centre region of the strip Rp-centre differ less than 20 N/mm².

6. Steel in accordance with any one of the preceding claims in the form of cold reduced, annealed and optionally further cold reduced strip or sheet wherein the average r-value is at least 1.3.

7. Method for manufacturing an annealed steel strip from the steel according to any one of claims 1-6, comprising the stages:
- hot-rolling comprising finish-rolling at a finish-rolling temperature and coiling at a coiling temperature;
- pickling;
- cold-rolling;
- annealing, preferably, continuous annealing, and optionally further cold rolling, preferably with a reduction of at least 0.6 %
wherein the finish-rolling temperature is selected above Ar₃-10 °C and the coiling temperature is selected below 700 °C.

8. Method according to claim 7, wherein the finish-rolling temperature is selected above 825 °C and the coiling temperature below 690 °C.

9. Method according to claim 7 or claim 8, wherein the finish-rolling temperature is selected at 900 ± 30 °C and the coiling temperature at 670 °C ± 20 °C.

10. Method according to claim 7, 8 or 9 wherein the total cold reduction before annealing is 85 % or more.

11. Method in accordance with anyone of claims 7-10, wherein further cold rolling after annealing is carried out with a reduction of> 5 %.

12. Method in accordance with claim 11 wherein further cold rolling after annealing is carried out with a reduction of 10-20 %.

13. Use of the steel in accordance with anyone of claims 1-6, or a steel strip obtained in the method in accordance with anyone of claims 7-12 for stretching, deep-drawing and drawing and wall-ironing applications.

14. Steel in accordance with anyone of claims 1-6, or obtained in a method in accordance with anyone of claims 713, provided with one or more coatings selected from the group of coatings comprising Sn, Cr, lacquer, organic coating, polymer and combinations thereof on one or both sides of the strip or sheet.

15. Stretched, deep drawn or drawn and wall ironed product made from steel according to any one of claims 1-6 or claim 14 or from steel obtained by the method or use according to any one of claims 7-13.

## Patentansprüche

1. Stahl in Form eines kaltreduzierten, vergüteten und wahlweise weiter kaltreduzierten Bleches oder Bandes mit folgender chemischen Zusammensetzung:
| Element | Minimum* | Maximum* |
|---|---|---|
| C | | 40 |
| Mn | 140 | 250 |
| P | | 20 |
| S | | 20 |
| Si | | 30 |
| N ppm | | 30 |
| Al** | | 50 |
| B ppm | 5 | 50 |
| Cu | | 40 |
| Sn | | 10 |
| Cr | | 40 |
| Ni | | 40 |
| Mo | | 10 |
| | | |
|---|---|---|
| * in 0,001 Gewichtprozent, wenn nicht anders angezeigt | | |
| ** säurelöslich | | |
mit dem Rest Fe und unvermeidbaren Unreinheiten, wobei 0,4 ≤ B / N ≤ 1,2, wobei die Korngröße in einem Kantenbereich des Streifens Gs-Kante und die Korngröße in einem Mittelbereich des Streifens Gs-Mitte weniger als 0,5 ASTM Einheiten abweicht.

2. Stahl nach Anspruch 1 mit folgender chemischen Zusammensetzung:
| Element | Minimum* | Maximum* |
|---|---|---|
| C | 10 | 40 |
| Mn | 140 | 200 |
| P | | 20 |
| S | | 20, vorzugsweise 10 |
| Si | | 30 |
| N ppm | | 25 |
| Al** | 15 | 35 |
| B ppm | 8 | 25 |
| Cu | | 40 |
| Sn | | 10 |
| Cr | | 40 |
| Ni | | 40 |
| Mo | | 10 |
| | | |
|---|---|---|
| * in 0,001 Gewichtprozent, wenn nicht anders angezeigt | | |
| ** säurelöslich | | |

3. Stahl nach Anspruch 1 oder Anspruch 2, worin für die folgenden Elemente die folgenden Standardwerte beachtet werden:
| Element | Standard* ± 30% |
|---|---|
| C | 20 |
| Mn | 160 |
| N ppm | 20 |
| Al** | 25 |
| B ppm | 0,8. N |
| | |
|---|---|
| * in 0,001 Gewichtprozent, wenn nicht anders angezeigt | |
| ** säurelöslich | |

4. Stahl nach einem der vorhergehenden Ansprüche in Form eines kaltreduzierten, vergüteten und wahlweise weiter kaltreduzierten Streifen oder Bleches, worin der r-Wert in einem Kantenbereich des Streifens r-Kante und der r-Wert in einem Mittelbereich des Bleches r-Mitte weniger als 0,2 Einheiten, vorzugsweise weniger als 0,1 Einheiten abweichen.

5. Stahl nach einem der vorhergehenden Ansprüche in Form eines kaltreduzierten, vergüteten und wahlweise weiter kaltreduzierten Streifens oder Bleches, worin der Fließpunkt in einem Kantenbereich des Streifens Rp-Kante und der Fließpunkt in einem Mittelbereich des Streifens Rp-Mitte weniger als 20 N/mm² abweicht.

6. Stahl nach einem der vorhergehenden Ansprüche in Form eines kaltreduzierten, vergüteten und wahlweise weiter kaltreduzierten Streifens oder Bleches, worin der durchschnittliche r-Wert wenigstens 1,3 beträgt.

7. Verfahren zur Herstellung eines vergüteten Stahlstreifens nach einem der Ansprüche 1 bis 6, das folgende Schritte umfaßt:
- Warmwalzen mit Fertigwalzen bei einer Fertigwalztemperatur und Wickeln bei einer Wickeltemperatur;
- Gelbbrennen;
- Kaltwalzen;
- Vergüten, vorzugsweise kontinuierliches Vergüten, und wahlweise weiteres Kaltwalzen, vorzugsweise mit einer Reduktion von wenigstens 0,6%,
wobei die Fertigwalztemperatur oberhalb von Ar₃-10 ° C und die Wickeltemperatur unterhalb von 700 °C gewählt wird.

8. Verfahren nach Anspruch 7, worin die Fertigwalztemperatur oberhalb von 825 °C und die Wickeltemperatur unterhalb von 690 °C gewählt wird.

9. Verfahren nach Anspruch 7 oder 8, worin die Fertigwalztemperatur bei 900 ± 30 °C und die Wickeltemperatur bei 670 °C ± 20 °C gewählt wird.

10. Verfahren nach Anspruch 7, 8 oder 9, worin die gesamte Kaltreduktion vor dem Vergüten 85% oder mehr beträgt.

11. Verfahren nach einem der vorhergehenden Ansprüche 7 bis 10, worin ein weiteres Kaltwalzen nach dem Vergüten mit einer Reduktion von > 5% durchgeführt wird.

12. Verfahren nach Anspruch 11, worin ein weiters Kaltwalzen nach dem Vergüten mit einer Reduktion von 10 bis 20% durchgeführt wird.

13. Verwendung von Stahl nach einem der Ansprüche 1 bis 6, oder einem Stahlstreifen, der mit einem Verfahren nach einem der Ansprüche 7 bis 12 hergestellt wurde, in Ausbreitungs-, Tiefzieh- und Zieh- und Wand-Abstreckziehanwendungen.

14. Stahl nach einem der Ansprüche 1 bis 6, oder der mit einem Verfahren nach einem der Ansprüche 7 bis 13 hergestellt wurde, der eine oder mehrere Beschichtungen, die aus der Gruppe von Beschichtungen, die Sn, Cr, Lack, organische Beschichtungen, Polymere und Kombinationen von diesen umfaßt, an einer oder an beiden Seiten des Streifens oder Blechen aufweist.

15. Ausgebreitetes, tiefgezogenes oder gezogenes und wandabstreckgezogenes Erzeugnis, das aus Stahl nach einem der Ansprüche 1 bis 6 oder aus Stahl, der mit einem Verfahren nach einem der Ansprüche 7 bis 13 erzeugt wurde, hergestellt wurde.

## Revendications

1. Acier sous forme de feuille ou bande façonnée à froid, recuite et éventuellement de nouveau façonnée à froid présentant une composition chimique :
| Elément | Min* | Max* |
|---|---|---|
| C | | 40 |
| Mn | 140 | 250 |
| P | | 20 |
| S | | 20 |
| Si | | 30 |
| N ppm | | 30 |
| Al** | | 50 |
| B ppm | 5 | 50 |
| Cu | | 40 |
| Sn | | 10 |
| Cr | | 40 |
| Ni | | 40 |
| Mo | | 10 |
| | | |
|---|---|---|
| * en 0,001 % en poids sauf indication contraire | | |
| ** soluble dans un acide | | |
le reste étant constitué de Fe et d'impuretés inévitables, dans lequel 0,4 ≤ B/N ≤ 1,2, dans lequel la taille de grain dans une zone de bord de la bande TG-bord et la taille de grain dans une zone centrale de la bande TG-centre diffèrent de moins de 0,5 unités ASTM.

2. Acier selon la revendication 1 présentant une composition chimique :
| Elément | Min* | Max* |
|---|---|---|
| C | 10 | 40 |
| Mn | 140 | 200 |
| P | | 20 |
| S | | 20, de préf. 10 |
| Si | | 30 |
| N ppm | | 25 |
| Al** | 15 | 35 |
| B ppm | 8 | 25 |
| Cu | | 40 |
| Sn | | 10 |
| Cr | | 40 |
| Ni | | 40 |
| Mo | | 10 |
| | | |
|---|---|---|
| * en 0,001 % en poids sauf indication contraire | | |
| ** soluble dans un acide | | |

3. Acier selon la revendication 1 ou 2, dans lequel, pour les éléments suivants, les valeurs standard suivantes sont respectées :
| Elément | Standard* ± 30 % |
|---|---|
| C | 20 |
| Mn | 160 |
| N ppm | 20 |
| Al** | 25 |
| B ppm | 0,8 . N |
| | |
|---|---|
| * en 0,001 % en poids sauf indication contraire | |
| ** soluble dans un acide | |

4. Acier selon l'une quelconque des revendications précédentes sous forme de bande ou feuille façonnée à froid, recuite et éventuellement de nouveau façonnée à froid dans lequel le coefficient r dans une zone de bord de la bande r-bord et le coefficient r dans une zone centrale de la bande r-centre diffèrent de moins de 0,2 unité, de préférence de moins de 0,1 unité.

5. Acier selon l'une quelconque des revendications précédentes sous forme de bande ou feuille façonnée à froid, recuite et éventuellement de nouveau façonnée à froid dans lequel la Limite d'Elasticité dans une zone de bord de la bande L-bord et la Limite d'Elasticité dans une zone centrale de la bande L-centre diffèrent de moins de 20 N/mm².

6. Acier selon l'une quelconque des revendications précédentes sous forme de bande ou feuille façonnée à froid, recuite et éventuellement de nouveau façonnée à froid dans lequel le coefficient r moyen vaut au moins 1,3.

7. Procédé de fabrication d'une bande d'acier recuit à partir de l'acier revendiqué dans l'une quelconque des revendications 1 à 6, comprenant les étapes de :
- laminage à chaud comprenant un finissage au laminoir à une température de finissage au laminoir et un bobinage à une température de bobinage;
- décapage;
- laminage à froid;
- recuit, de préférence recuit continu, et éventuellement laminage à froid supplémentaire, de préférence avec une réduction d'au moins 0,6 %
dans lequel la température de finissage au laminoir est choisie au-dessus de Ar3-10 °C et la température de bobinage est choisie en-dessous de 700 °C.

8. Procédé selon la revendication 7, dans lequel la température de finissage au laminoir est choisie au-dessus de 825 °C et la température de bobinage est choisie en-dessous de 690 °C.

9. Procédé selon la revendication 7 ou 8, dans lequel la température de finissage au laminoir est choisie à 900 ± 30 °C et la température de bobinage est choisie à 670 °C ± 20 °C.

10. Procédé selon l'une quelconque des revendications 7 à 9, dans lequel la réduction totale à froid avant recuit est de 85 % ou plus.

11. Procédé selon l'une quelconque des revendications 7 à 10, dans lequel le laminage à froid supplémentaire après recuit est exécuté avec une réduction supérieure à 5 %.

12. Procédé selon la revendication 11, dans lequel le laminage à froid supplémentaire après recuit est exécuté avec une réduction de 10-20 %.

13. Utilisation de l'acier revendiqué dans l'une quelconque des revendications 1 à 6, ou d'une bande d'acier obtenue avec le procédé revendiqué dans l'une quelconque des revendications 7 à 12, pour des applications d'étirement, d'emboutissage profond et d'emboutissage-étirage.

14. Acier selon l'une quelconque des revendications 1 à 6, ou obtenu avec un procédé selon l'une quelconque des revendications 7 à 13, muni d'un revêtement ou plus choisi parmi le groupe de revêtements comprenant Sn, Cr, de la laque, un revêtement organique, un polymère et des combinaisons de ceux-ci sur une ou les deux faces de la bande ou feuille.

15. Produit étiré, embouti ou embouti-étiré constitué d'acier selon l'une quelconque des revendications 1 à 6 ou 14 ou d'acier obtenu par le procédé ou l'utilisation selon l'une quelconque des revendications 7 à 13.
